

# UNITED STATES PATENT OFFICE.

JOHN J. DAVOREN, OF DENVER, COLORADO, ASSIGNOR OF ONE-HALF TO WILLIAM T. DAVOREN, OF DENVER, COLORADO.

## COMPOSITION OF MATTER.

1,024,561.

Specification of Letters Patent. Patented Apr. 30, 1912.

No Drawing.

Application filed May 26, 1911. Serial No. 629,732.

*To all whom it may concern:*

Be it known that I, JOHN J. DAVOREN, a citizen of the United States of America, residing at Denver, in the county of Denver and State of Colorado, have invented certain new and useful Improvements in Composition of Matter, of which the following is a specification.

My invention relates to a new composition 10 of matter to be used principally in the manufacture of machine parts and its object is to provide a metallic substance in which softness is combined with tenacity.

My composition consists in its preferred 15 form of the following ingredients combined in the proportions stated viz:—

|               |                      |
|---------------|----------------------|
| Lead          | 50 pounds.           |
| Copper        | 50 pounds.           |
| Arsenic       | $\frac{1}{2}$ pound. |
| 20 Phosphorus | 1 ounce.             |

The above component parts are combined by melting the metals and adding the non-metallic elements to the molten mass, after 25 which the latter is poured into a suitable mold. The substance thus produced is ready for instant use when cooled.

While the above described composition 30 may be employed for many different purposes, it is particularly adapted to be used in the manufacture of machine parts which are in constant frictional contact with each other or with parts made of different material, as for example the linings of journal 35 bearings.

I wish it understood that while a compound of the above enumerated ingredients in the proportions stated has produced the most satisfactory results, brass, bronze or any other alloy may be substituted for the 40 copper, and to adapt the composition to different purposes the proportions of the constituent elements may be varied.

The phosphorus which is added to the mixture to render the metals more fusible, 45 is essential in the production of the alloy, but inasmuch as the arsenic is used only when it is desired to produce an alloy of finer grain, the same may be omitted under ordinary circumstances.

What I claim and desire to secure by Letters-Patent is:

1. The herein described composition of matter consisting of copper, lead and phosphorus.
2. The herein described composition of matter consisting of copper fifty pounds, lead fifty pounds and phosphorus one ounce.
3. The herein described composition of matter consisting of copper and lead in 55 equal proportions and phosphorus.

In testimony whereof I have affixed my signature in presence of two witnesses.

JOHN J. DAVOREN.

Witnesses:

G. J. ROLLANDET,  
L. RHOADES.